



US005441555A

**United States Patent** [19]

Matthews et al.

[11] **Patent Number:** 5,441,555[45] **Date of Patent:** Aug. 15, 1995[54] **POWDER METALLURGY COMPOSITIONS**[75] Inventors: Paul Matthews; Thomas Pelletier, II,  
both of Flemington, N.J.[73] Assignee: United States Bronze Powders, Inc.,  
Flemington, N.J.

[21] Appl. No.: 279,223

[22] Filed: Jul. 22, 1994

**Related U.S. Application Data**[63] Continuation of Ser. No. 930,698, filed as  
PCT/GB91/00351, Mar. 6, 1991, abandoned.[30] **Foreign Application Priority Data**Mar. 6, 1990 [GB] United Kingdom ..... 9005036  
Jan. 29, 1991 [GB] United Kingdom ..... 9101829[51] **Int. Cl.<sup>6</sup>** ..... C22C 9/02; C22C 9/04[52] **U.S. Cl.** ..... 75/255; 75/252;  
420/470; 420/477; 420/499[58] **Field of Search** ..... 75/247, 252, 255;  
420/470, 474, 477, 499[56] **References Cited****U.S. PATENT DOCUMENTS**

- 1,421,471 7/1922 Heskett ..... 75/255  
 2,286,237 6/1942 Shaw et al. ..... 75/255  
 2,467,675 4/1949 Kurtz et al. ..... 75/255  
 3,370,942 7/1964 Inoue ..... 75/134  
 3,790,352 2/1974 Niimi et al. ..... 75/247  
 3,805,000 4/1974 Roy ..... 200/144 B  
 3,832,156 8/1974 Wilson et al. ..... 75/0.5 B  
 3,948,652 4/1976 Schreiner et al. ..... 75/170  
 4,014,688 3/1977 Schreiner et al. ..... 75/123 B  
 4,014,698 3/1977 Schreiner et al. ..... 75/129  
 4,169,730 10/1979 Matthews et al. ..... 75/157  
 4,172,720 10/1979 Megelas ..... 75/251  
 4,537,743 8/1985 Yamanaka et al. ..... 419/38  
 4,540,437 9/1985 Patel ..... 75/251  
 4,551,395 11/1985 Lloyd ..... 428/677  
 4,708,739 11/1987 Kellie et al. ..... 75/76  
 4,770,723 9/1988 Sagawa et al. ..... 75/255  
 4,834,794 5/1989 Yagi et al. ..... 75/255  
 4,879,094 11/1989 Rushton ..... 420/476  
 4,920,020 4/1990 Strauven et al. ..... 75/255  
 4,981,513 1/1991 Ghandehari ..... 75/255  
 5,137,685 8/1992 McDevitt et al. ..... 420/499  
 5,167,726 12/1992 LoFacono et al. ..... 420/499  
 5,354,352 10/1994 Seki et al. ..... 75/247

**FOREIGN PATENT DOCUMENTS**

- 692687 8/1964 Canada ..... 75/255  
 0083200 12/1982 European Pat. Off. .  
 0224619 11/1985 European Pat. Off. .  
 165872 12/1985 European Pat. Off. ..... 75/255  
 3829250 3/1990 Germany .  
 56-142839 11/1981 Japan ..... 420/470  
 250721 2/1925 United Kingdom .  
 581903 5/1944 United Kingdom .  
 615172 7/1947 United Kingdom .  
 901026 5/1958 United Kingdom .  
 1000651 11/1965 United Kingdom .  
 1162573 8/1969 United Kingdom .  
 1390212 4/1975 United Kingdom .  
 1518781 7/1978 United Kingdom .  
 2211206 6/1989 United Kingdom .  
 655742 4/1979 U.S.S.R. ..... 75/255

**OTHER PUBLICATIONS**Chem Abstr., vol. 105, No. 10, 83631s (Katsuhiro et al.)  
Imon, (Japan) 1986, 58(6), 449-454.

Chem. Abstr., vol. 97, No. 24, 202192 (Hitachi Chemical Co.).

Chem. Abstr., vol. 96, No. 16, 128144 (Hitachi Chemical Co.).

Primary Examiner—George Wyszomierski  
Attorney, Agent, or Firm—Woodcock Washburn Kurtz  
Mackiewicz & Norris[57] **ABSTRACT**

Lead-free metallurgy powder for use in manufacturing a shaped bronze part by powder metallurgy techniques which consists essentially of a substantially homogeneous blend of about 90 parts copper, about 10 parts tin and an amount of bismuth in the range from an amount effective to improve the machinability of the shaped bronze part up to about 5% weight are disclosed. Lead-free metallurgy powder for use in manufacturing a shaped bronze part by powder metallurgy techniques which consists essentially of a substantially homogeneous blend of about 70-90 parts copper, about 10-30 parts zinc and an amount of bismuth in the range from an amount effective to improve the machinability of the shaped bronze part up to about 5% weight are also disclosed.

22 Claims, No Drawings

## POWDER METALLURGY COMPOSITIONS

## CROSS REFERENCE TO RELATED PATENT APPLICATIONS

This application is a File Wrapper Continuation Application of U.S. application Ser. No. 07/930,698 filed as PCT/GB91/00351, Mar. 6, 1991, abandoned.

## DESCRIPTION

This invention relates to powder metallurgy compositions containing elemental and/or prealloyed non-ferrous metal powders, organic lubricants, and with or without flake graphite additives. For example pre-blended bronze compositions are commonly used for self-lubricating bearings and bushings, oil impregnated bearings for motor use, household appliances, tape recorders, video cassette recorders etc. In commercial powder metallurgy practices, powdered metals are convened into a metal article having virtually any desired shape.

The metal powder is firstly compressed in a die to form a "green" preform or compact having the general shape of the die. The compact is then sintered at an elevated temperature to fuse the individual metal particles together into a sintered metal part having a useful strength and yet still retaining the general shape of the die in which the compact was made. Metal powders utilized in such processes are generally pure metals, OR alloys or blends of these, and sintering will yield a part having between 60% and 95% of the theoretical density. If particularly high density low porosity is required, then a process such as a hot isostatic pressing will be utilized instead of sintering. Bronze alloys used in such processes comprise a blend of approximately 10% of tin powder and 90% of copper powder and according to one common practice the sintering conditions for the bronze alloy are controlled that a predetermined degree of porosity remains in the sintered part. Such parts can then be impregnated with oil under pressure of vacuum to form a so-called permanently lubricated bearing or component and these parts have found wide application in bearings and motor components in consumer products and eliminate the need for periodic lubrication of these parts during the useful life of the product.

Solid lubricants can also be included and these are typically waxes, metallic/non-metallic stearates, graphite, lead alloy, molybdenum disulfide and tungsten disulfide as well as many other additives, but the powders produced for use in powder metallurgy have typically been commercially pure grades of copper powder and tin powder which are then admixed in the desirable quantities.

For many metallurgical purposes, however, the resulting sintered product has to be capable of being machined that is to say, it must be capable of being machined without either "tearing" the surface being machined to leave a "rough" surface or without unduly blunting or binding with the tools concerned. It is the common practice for a proportion of lead up to 10% to be included by way of a solid lubricant to aid and improve the machineability of the resulting product.

Lead is, however, a toxic substance and the use of lead in the production of alloys is surrounded by legislation and expensive control procedures. Furthermore, the lead phase in copper lead alloys can be affected by corrosive attacks with hot organic or mineral oil; when

the temperature of such an alloy rises; for example in service it has been known that the oil can break down to form peroxides and organic gases which effect a degree of leaching on the lead phase within the alloy. If this leaching progresses to any extent, the component if it is a bearing or structural component, may eventually malfunction or fail.

Accordingly, there is considerable advantage in reducing, or if possible, eliminating the contents of lead within powder metallurgy compositions.

According to one aspect of the present invention, therefore, there is provided a powder composition suitable for use in powder metallurgy in which composition the lead content has been substituted by an effective amount of bismuth.

In one aspect of the present invention, the proportion of bismuth is within the range of 35% to 65% of the proportion of lead that it replaces. In a further aspect of the present invention, the powder composition may be bronze powder and the bismuth may be present in an amount of up to 5% by weight.

The bismuth may be present as an elemental powder or may be prealloyed with another constituent of the powder composition. For example, where the powder composition is bronze powder, the bismuth may be prealloyed either with tin as a bismuth tin alloy in powder form or with copper as a copper bismuth alloy in powder form.

In a further aspect of the present invention a proportion of lubricant may be included to improve further the machineability of the resulting alloy. A typical lubricant is graphite which may be included in an amount of 0.1% to 0.9% by weight. Other lubricants are low density polyalkylenes such as that commercially available under the trade name COATHYLENE; stearic acid and zinc stearate which may be included separately or in combination.

In a powder metallurgy bronze powder in accordance with the present invention, lead may be replaced by approximately one half of its quantity of bismuth to obtain the same degree of machineability, i.e. in general terms 2% of bismuth could replace a 4% on the weight of bronze powder of lead.

Investigations have established that bismuth has no known toxicity. Bismuth is non-toxic and its developing or proliferating uses in pharmaceuticals, cancer-reducing therapy, X-ray opaque surgical implants and other medical equipment indicate that bismuth, while not only more efficient in improving the machineability, also has low or nil toxicity.

The present invention also includes products when manufactured by powder metallurgy techniques using the powder in accordance with the present invention.

Following is a description by way of example only of methods of carrying the invention into effect.

## EXAMPLE 1

A powder metallurgic bronze powder system comprised 90% of elemental copper powder, 10% of elemental tin powder and 0.75% of lubricant on the weight of the tin and copper. A number of elemental conditions of both bismuth and lead were made in various percentages to the basic composition and the results are set out in Table 1. In order to evaluate the effectiveness of each addition, test specimens were made and underwent a standard drilling test. All reported data from this test is based on an average of multiple drilling tests and is

reported in standardised inches per minute. All test specimens were standard MPIF transverse rupture bars pressed to a reported green density. All data in Table 1 reflects test specimens sintered at 1520° F. for a time of 15 minutes under a dissociated ammonia atmosphere (75% H<sub>2</sub>, 25% N<sub>2</sub>).

TABLE 1

| Elemental                      | Green Density         | Comparative Tests: Drilling Rate (inches/minute) |     |      |      |
|--------------------------------|-----------------------|--------------------------------------------------|-----|------|------|
|                                |                       | 0                                                | 1   | 3    | 5    |
| Bronze (No Pb or Bi Additions) | 6.0 g/cm <sup>3</sup> | 0.9                                              | —   | —    | —    |
| Bronze + Bi                    | 6.5 g/cm <sup>3</sup> | 1.2                                              | —   | —    | —    |
| Bronze + Pb                    | 6.0 g/cm <sup>3</sup> | —                                                | 8.6 | 14.0 | 8.9  |
|                                | 6.5 g/cm <sup>3</sup> | —                                                | 9.8 | 11.7 | 4.3  |
|                                | 6.0 g/cm <sup>3</sup> | —                                                | 9.5 | 22.2 | 13.0 |
|                                | 6.5 g/cm <sup>3</sup> | —                                                | 8.2 | 19.0 | 7.7  |

In Table 1 it will be seen that a percentage of 1% of bismuth produces comparable drilling time with the corresponding figures for lead.

EXAMPLE 2

Copper bismuth was prealloyed, atomized and powdered bronze compositions were prepared having the compositions containing 10% tin powder. Sintered test bars were prepared and drilled and the drilling time

All test specimens in Table 4 were sintered at 1600° F. for a total time of 45 minutes in a dNH<sub>3</sub> atmosphere.

TABLE 3

| 5                  | Total                 | Drilling time (in/min) |      |     |      |     |
|--------------------|-----------------------|------------------------|------|-----|------|-----|
|                    |                       | % Bi                   | 0    | .01 | .03  | .05 |
| 70/30 Brass        | 7.3 g/cm <sup>3</sup> | .25                    | .43  | .53 | .45  |     |
| 85/15 Brass        | 7.6 g/cm <sup>3</sup> | .36                    | .43  | .49 | .51  |     |
| 90/10 Brass        | 7.8 g/cm <sup>3</sup> | .30                    | .25  | .66 | .61  |     |
| 70/30 Leaded Brass | 7.3 g/cm <sup>3</sup> | 2.78                   | 4.68 | .6  | 4.24 |     |
| 80/20 Leaded Brass | 7.6 g/cm <sup>3</sup> | 3.46                   | 4.80 | .53 | 3.00 |     |

EXAMPLE 4

15 A bronze powder containing 90% copper and 10% tin was provided with the further addition of 0.5% by weight on the weight of the copper, tin, of bismuth. Selected additions of carbon graphite, coathylene lubricant, stearic acid or zinc stearate were added. Sintered test bars were prepared and then test drilled. The drilling time in inches per minute through a  $\frac{1}{4}$  inch thick sintered bar of given density at a constant drill bit speed and a drill unit false free fall weight, i.e. no spring retainer or varying physical force.

All test data set out in the following table reflects test specimens pressed to a green density of 6.0 g/cm<sup>3</sup>, and sintered at 1520° F. for a time of 15 minutes under a dissociated ammonia atmosphere (75% H<sub>2</sub>, 25% N<sub>2</sub>).

TABLE 4

| % GRAPHITE | % COATHYLENE | % STEARIC ACID | % ZINC STEARATE | DRILLING SPEED (IN MINS) |
|------------|--------------|----------------|-----------------|--------------------------|
| 0.00       | 0.00         | 0.00           | 0.75            | 5.4                      |
| 0.00       | 0.50         | 0.25           | 0.00            | 5.0                      |
| 0.10       | 0.00         | 0.00           | 0.75            | 11.6                     |
| 0.10       | 0.50         | 0.25           | 0.00            | 10.1                     |
| 0.30       | 0.00         | 0.00           | 0.75            | 18.8                     |
| 0.30       | 0.50         | 0.25           | 0.00            | 15.3                     |
| 0.50       | 0.00         | 0.00           | 0.75            | 17.1                     |
| 0.50       | 0.50         | 0.25           | 0.00            | 32.8                     |

given is the actual time converted into inches per minute required to drill a 3/16" hole completely through a  $\frac{1}{4}$  thick sintered bar at a constant drill bit speed and drill unit false weight free fall, i.e. no spring retainer or varying physical force.

TABLE 2

| Green Density g/cm <sup>3</sup> | Drilling Rate (inches/minute) vs. Bi % |     |     |     |     |     |
|---------------------------------|----------------------------------------|-----|-----|-----|-----|-----|
|                                 | % Bi                                   |     |     |     |     |     |
| 0                               | 0.5                                    | 1.0 | 2.0 | 3.0 | 5.0 |     |
| 6.0                             | 0.9                                    | 4.2 | 7.9 | 8.2 | *   | *   |
| 6.5                             | 1.2                                    | 4.1 | 6.6 | 8.2 | *   | *   |
| 7.5                             | 0.2                                    | —   | 8.4 | —   | 6.6 | 4.1 |
| 7.9                             | **                                     | —   | 8.3 | —   | 8.5 | 6.2 |

\*Prealloyed Cu/Bi powder physical properties prevented practical compacting of test bars.

\*\*Standard Copper/Tin powder reference blend could not be practically compacted to 7.9 g/cm<sup>3</sup> density.

It will be seen that the addition of quantities of bismuth produced improvements in the machineability with increasing green density.

EXAMPLE 3

#### Additions to P/M Brasses

In order to evaluate the effectiveness of Bi additions to brass machineability characteristics, additions were made to both Non-leaded and Leaded brasses. All testing was done in accordance with the testing procedure mentioned earlier.

45 A standard bronze composition comprising 90% elemental copper powder, 10% elemental tin powder, and 0.75% lubricant, had a drilling rate of 0.9 inches per minutes when processed under the same conditions.

The above tests show significant increases in the drilling rate, up to 36 times the standard rate.

We claim:

1. A metallurgy powder for use in manufacturing a shaped bronze part by powder metallurgy techniques, the powder consisting essentially of a substantially homogeneous blend of about 90 parts copper, about 10 parts tin and an amount of bismuth in the range from an amount effective to improve the machinability of the shaped bronze part up to about 5% weight, the powder being substantially free of lead.
2. The metallurgy powder of claim 1 wherein the bismuth is included as an elemental powder.
3. The metallurgy powder of claim 1 wherein the bismuth is present as a pre-alloy with copper.
4. The metallurgy powder of claim 1 wherein the bismuth is pre-alloyed with the tin.
5. The metallurgy powder of claim 1 further consisting of a lubricant.
6. The metallurgy powder of claim 1 further consisting of a lubricant selected from the group consisting of graphite, low density polyalkylenes, stearic acid and zinc stearate.

7. The metallurgy powder of claim 1 further consisting of 0.1%-0.9% wt graphite.

8. A metallurgy powder for use in manufacturing a shaped brass part by powder metallurgy techniques, the powder consisting essentially of a substantially homogeneous blend of about 70-90 parts copper, about 10-30 parts zinc and an amount of bismuth in the range from an amount effective to improve the machinability of the shaped brass part up to about 5% weight, the powder being substantially free of lead.

9. The metallurgy powder of claim 8 wherein the bismuth is included as an elemental powder.

10. The metallurgy powder of claim 8 wherein the bismuth is present as a pre-alloy with copper.

11. The metallurgy powder of claim 8 wherein the bismuth is pre-alloyed with the zinc.

12. The metallurgy powder of claim 8 further consisting of a lubricant.

13. The metallurgy powder of claim 8 further consisting of a lubricant selected from the group consisting of graphite, low density polyalkylenes, stearic acid and zinc stearate.

14. The metallurgy powder of claim 8 further consisting of 0.1%-0.9% wt graphite.

15. A metallurgy powder for use in manufacturing a shaped bronze part by powder metallurgy techniques, the powder consisting essentially of a substantially homogeneous blend that comprises about 90 parts copper, about 10 parts tin and an amount of bismuth in the range from an amount effective to improve the machinability of the shaped bronze part up to about 5% weight,

wherein the powder is substantially free of lead, and the total weight of the powder consists of copper and tin except for up to about 5.9%.

16. The metallurgy powder of claim 15 further consisting of a lubricant.

17. The metallurgy powder of claim 15 further consisting of a lubricant selected from the group consisting of graphite, low density polyalkylenes, stearic acid and zinc stearate.

18. The metallurgy powder of claim 15 further consisting of 0.1%-0.9% wt graphite.

19. A metallurgy powder for use in manufacturing a shaped brass part by powder metallurgy techniques, the powder consisting essentially of a substantially homogeneous blend that comprises about 70-90 parts copper, about 10-30 parts zinc and an amount of bismuth in the range from an amount effective to improve the machinability of the shaped brass part up to about 5% weight, wherein the powder is substantially free of lead, and the total weight of the powder consists of copper and zinc except for up to about 5.9%.

20. The metallurgy powder of claim 19 further consisting of a lubricant.

21. The metallurgy powder of claim 19 further consisting of a lubricant selected from the group consisting of graphite, low density polyalkylenes, stearic acid and zinc stearate.

22. The metallurgy powder of claim 19 further consisting of 0.1%-0.9% wt graphite.

\* \* \* \* \*